

# UNITED STATES PATENT OFFICE.

OTTO RÖHM, OF DARMSTADT, GERMANY.

## PROCESS FOR THE MANUFACTURE OF IRON-LEATHER.

1,397,387.

Specification of Letters Patent. Patented Nov. 15, 1921.

No Drawing.

Application filed July 9, 1920. Serial No. 395,146.

To all whom it may concern:

Be it known that I, OTTO RÖHM, a citizen of the Free State of Wurttemberg, in the German Republic, residing at Darmstadt, 5 in the State of Hessa, Germany, have invented Improvements in and Relating to a Process for the Manufacture of Iron-Leather, (for which I have filed applications in Germany May 2, 1918; in Czechoslovakia 10 Aug. 19, 1919; in Austria Nov. 22, 1919; in Hungary Nov. 28, 1919; and in Spain March 30, 1920;); and I do hereby declare the following to be a full, clear, and exact description of the same.

15 My invention relates to a process for tawing or alutation of skins by means of silicate of iron, in which the skins are acted upon by solutions of iron salts and silicates together, *i. e.* in a single tawing bath.

20 Hitherto for the manufacture of iron-leather soluble iron salts for instance basic sulfate of iron or basic ferric chlorid have been used. It has also been proposed to first taw the skins with soluble iron salts and 25 then to put the iron-leather thus obtained in a solution containing (besides sebacic combinations) alkaline silicate. In proceeding in this way a part of the iron salt taken up by the skin is first precipitated again and 30 forms with the alkaline silicate an insoluble silicate of iron. The latter settles upon the skin which thereby becomes brittle.

According to the new process the skin is 35 acted upon by the silicate of iron during the colloidal state whereby a non brittle iron-leather is obtained in a simple and accelerated manner. To this end the skins during tawing with iron salts are brought 40 together with diluted solutions of water-glass.

If in carrying out this process a concentrated solution of water-glass of 36° Bé. would be added to a solution of an iron salt, such as ferric chlorid, a separation of 45 insoluble silicate of iron would take place at once and a tawing with this mixture would be impossible. If however the concentrated solution of water-glass is first diluted for instance with an 8-10 fold quantity of water and said solution of water-glass added to the solution of ferric chlorid, a separation of silicate of iron does not take place even if up to 4 parts of water-glass are added to one part of ferric-chlorid. 50 Moreover the deposit of silicate of iron

formed at the beginning of the process is perfectly dissolved again on stirring.

The solutions of silicate of iron thus obtained are, as stated above, especially adapted for the manufacture of iron-leather. 60 Against solutions of basic iron salts the said solutions of silicate of iron have the advantage that they very easily penetrate the skin or in other words very quickly taw.

The invention may also be carried out in 65 such a manner that the skin is first brought into the solution of iron salt and after the latter has penetrated the skin the desired quantity of solution of water-glass is slowly added to the same bath. In this way also 70 the forming of insoluble silicate of iron is prevented.

It has already been stated above that according to the new process up to 4 parts of water-glass may be used with 1 part of iron 75 salt. Depending upon the proportions used leather of different properties is obtained and the more water-glass is used in proportion to the iron salt the fuller and stronger 80 the leather.

To obtain iron-leather by means of silicate of iron one of the following processes may be used:

1. To taw 100 kg. of skins a clear solution of silicate of iron is prepared by adding a diluted solution of water-glass to a solution of 10 kg. ferric chlorid in 100 l. water. For instance 200-300 kg. of a 10% solution of concentrated water-glass is added and with this mixture the skins are tawed, 90 washed out, fatted if necessary, dried and dressed in a well known manner.

2. 100 kg. of skins are first placed in a solution of 10 kg. of ferric chlorid and 5 kg. of common salt in 100 l. water. After some time 200-300 kg. of a 10% solution of water-glass are slowly added to the constantly moving tawing bath. The moving is continued until the skin does not take up any more tawing matter. The leather is then 100 taken out, washed out with water, fatted if necessary, dried and dressed.

To further improve the properties of the iron-leather thus obtained the same measures may be taken as are used in the other tawing 105 processes by means of iron salts. Thus I have already earlier recognized the profit which may be obtained by combining the tawing by means of the usual iron salts with a tawing by means of formaldehyde. Ac- 110

cording to the present process also the tawing action will be improved by the use of aldehydes for instance formaldehyde and a specially resistant leather is obtained. The 5 aldehyde may be added during any desired stage of the process, *i. e.* before, during or after the tawing explained above.

If these improvements are to be used 2-3 kg. of formaldehyde may be added to the 10 example of the quantity of water-glass given above for the tawing of 100 kg. of skins. The formaldehyde tawing may however take place before or after the tawing with iron salts.

15 It may also be stated that before the tawing the skins may be pickled as is usual in tawing with chrome salts. Also the pickling acid may be added to the salt solutions described above. By the use of acid in this 20 form the tawing is accelerated and a specially smooth grain is obtained.

Having now described and ascertained the nature of my invention and the manner in which the same is to be performed I now 25 declare what I claim and desire to secure by Letters Patent of the United States is:

1. The herein described process for manufacturing iron-leather, consisting in subjecting the skins to a solution of iron salts, and 30 adding a diluted solution of water glass to said solution.

2. The herein described process for manufacturing iron leather, consisting in subjecting the skins to a solution of iron salts and then slowly adding a diluted solution of 35 water glass to said solution.

3. The process herein described for manufacturing iron leather, consisting in subjecting the skins to a tawing solution of silicate of iron obtained by mixing a solution of 40 iron salts with a diluted solution of water glass.

4. The herein described process for manufacturing iron leather, consisting in subjecting the skins to a tawing solution of iron 45 salts, adding a diluted solution of water glass to the tawing solution, and adding a solution of formaldehyde to the tawing solution.

5. The herein described process for manufacturing iron-leather, consisting in subjecting the skins to a solution of iron salts, and adding to said solution a solution of water glass and formaldehyde.

In testimony whereof, I have signed my 55 name to this specification in the presence of two subscribing witnesses.

DR. OTTO RÖHM.

Witnesses:

HUGO HAIG,  
D. WILHELM ANDRES.